

Jan. 31, 1967

L. T. COPPETA

3,300,879

MARK RESISTANT COATING

Filed March 30, 1965

|                                 | TRUE                                  | FALSE                                 |
|---------------------------------|---------------------------------------|---------------------------------------|
| 1 - Top coating if any not.     | <input type="checkbox"/>              | <input checked="" type="checkbox"/> 6 |
| 2 - Sci/ie mirror like.         | <input checked="" type="checkbox"/> 6 | <input type="checkbox"/>              |
| 3 - Ware too will, is metallic. | <input checked="" type="checkbox"/> 6 | <input type="checkbox"/>              |
| 4 - In Circu in Alum.           | <input type="checkbox"/>              | <input checked="" type="checkbox"/> 6 |

INVENTOR.

LEONARD T. COPPETA

BY

*Kenway, Jenney & Hildreth*

ATTORNEYS

# United States Patent Office

3,300,879  
Patented Jan. 31, 1967

## 1

3,300,879

### MARK RESISTANT COATING

Leonard Thomas Coppeta, North Andover, Mass., assignor to The Carter's Ink Company, Cambridge, Mass., a corporation of Massachusetts

Filed Mar. 30, 1965, Ser. No. 443,979  
1 Claim. (Cl. 35—48)

This invention relates to self-correcting testing devices, more particularly to a sheet for receiving test marks in a manner which indicates whether a given marking is correct.

The testing devices of this invention may be used in connection with numerous teaching programs which can utilize testing of the multichoice type. In these the student is given a question, or instructions requiring him to mark a score sheet in one or several areas according to the particular test pattern. Certain areas correspond to "right" answers, and others to "wrong" answers. The test is scored by tallying the number of right and wrong answers.

In the testing device of this invention the score sheet is designed to receive markings only in selected areas, which may correspond to either the right answer or the wrong answer, and the student is immediately apprised of whether his selection of a particular marking area is correct.

The score sheet of this invention is provided with visible marks defining the areas to be marked, the surfaces of a selected number of which are of sufficient roughness and high coefficient of friction to receive a mark from a given pencil or similar marking device, and the surfaces of the others are of sufficient smoothness and low coefficient of friction as not to pick up a mark from the same device.

It has been found that selected surface areas of a sheet may be rendered relatively less capable of being marked upon without substantially altering the appearance or feel of the surface sufficiently to designate to a casual observer which area is which. Preferably the base sheet will be paper having a smooth surface, such as a bond paper or other rag pulp or chemical wood pulp paper, which may be uncoated or surface sized.

Selective areas of the paper are rendered more mark resistant by the application of a coating of plastic, polymeric, or waxy material having surface properties that render it incapable of eliciting a mark from a soft lead pencil or similar device.

Many materials and formulations may be devised to behave in this manner, examples of which are given below. In general, the coating will make use of such materials as waxes, e.g., paraffinic hydrocarbon waxes, polyethylene, aluminum stearate, halogen substituted polyolefins, high molecular weight alcohols and esters, and other similar solid materials of a soft and waxy or unctuous nature capable of forming a coating having a smooth surface. In addition, various compatible modifiers, plasticizers and additives, commonly employed in materials of this nature may be incorporated.

By way of example the following coating compositions may be employed with entirely satisfactory results, the first of these being the presently preferred embodiment.

## 2

### Example I

| Ingredient:          | Percent by weight |
|----------------------|-------------------|
| Nuosperse 657        | 1.0               |
| EHEC-High            | 3.0               |
| Piccotex 120 Resin   | 7.0               |
| Aluminum stearate    | 12.0              |
| Isopar K             | 43.0              |
| Chlorothene NU       | 15.0              |
| Methyl ethyl ketone  | 15.0              |
| A-C Polyethylene 656 | 4.0               |

A solution of EHEC and Piccotex 120 in methyl ethyl ketone and Chlorothene is prepared and set aside. One-twelfth (1.0% of total formulation) of the aluminum stearate and the A-C Polyethylene 656 is dissolved in Isopar K at 160° F. This solution is allowed to cool to room temperature, whereupon the polyethylene forms a dispersion, and the remainder of the aluminum stearate is added with agitation. Finally, the solution of EHEC and the dispersion are combined and the paper is coated.

### Example II

| Ingredient:                 | Percent by weight |
|-----------------------------|-------------------|
| EHEC-High                   | 4.0               |
| Piccotex 120 Resin          | 12.0              |
| Isopar K                    | 34.0              |
| Chlorothene NU              | 29.0              |
| Microthene 200 Polyethylene | 16.0              |
| A-C Polyethylene 656        | 5.0               |

This formulation is processed in the same manner as in Example I. The EHEC and Piccotex are dissolved in the Chlorothene, and the Microthene and A-C Polyethylene 656 are dispersed in the Isopar.

### Example III

| Ingredient:          | Percent by weight |
|----------------------|-------------------|
| EHEC-High            | 2.0               |
| Piccotex 120 Resin   | 15.0              |
| Isopar K             | 30.0              |
| Chlorothene          | 30.0              |
| Nuosperse 657        | 1.0               |
| Stearic acid         | 2.0               |
| Zinc stearate        | 5.0               |
| Microthene 200       | 12.0              |
| A-C Polyethylene 656 | 3.0               |

This formulation is processed in the same manner as in Example I. The EHEC and Piccotex are dissolved in the Chlorothene, and the Microthene and A-C Polyethylene 656 are dispersed in the Isopar. Zinc stearate and stearic acid are used in lieu of aluminum stearate.

### Example IV

| Ingredient:          | Percent by weight |
|----------------------|-------------------|
| A-C Polyethylene 656 | 40                |
| Tergitol NPX         | 10                |
| Potassium hydroxide  | .6                |
| Water                | 49.4              |

The ingredients are combined and mixed together. In the foregoing examples:

Nuosperse 657 is a combination wetting, dispersing, and anti-settling agent produced by the Nuodex Products Division of Heyden Newport Chemical Corporation.

EHEC-High is a high viscosity—125 to 250 centipoises—ethyl hydroxy ethyl cellulose, manufactured by Hercules Powder Company.

Piccotex 120 is an aromatic, thermoplastic styrene copolymer resin, having a softening point, ball-and-ring, of 120° C., produced by Pennsylvania Industrial Chemical Corporation.

Isopar K is a synthetic petroleum hydrocarbon having a chemical composition that is about 95 percent isoparaffinic (branched), sold by the Humble Oil & Refining Company.

Chlorothene NU is a specially inhibited 1,1,1-trichloroethane, prepared by The Dow Chemical Company.

The A-C Polyethylene is an oxidized, emulsifiable polyethylene produced by Allied Chemical Corporation.

Microthene 200 is a polyethylene powder produced by U.S. Industrial Chemicals Company.

Tergitol NPX is a nonyl phenyl polyethylene glycol containing 10.5 moles of ethylene oxide, an "all-purpose" non-ionic detergent and wetting agent produced by Union Carbide Chemicals Company.

A testing device embodying this invention is shown in the accompanying drawing in which

FIG. 1 is a plan view.

The sheet 2, preferably formed of bond paper of 16-28 lbs. per ream (500 sheets 17" x 22") is imprinted with test questions which call for answers to be applied by marking one or another of several areas 4. Certain of these, 6, are provided with a substantially invisible coating of a mark resistant composition, such as that described in Example I above. Preferably the material is applied to a thickness of four-tenths of a mil or more, conveniently by silk screening the coating composition onto the paper and then allowing it to dry.

In use the coated areas will resist a mark from a soft lead pencil such as that designated "Dixon," Andel black 195.

Other suitable paper bases include white offset book

paper, typically weighing 50-100 lbs. per ream (500 sheets 25" x 38"), text paper, or ledger paper, which may be of rag or chemical wood pulp. These papers have a surface appearance similar to that of the coating, and render the coated areas unobvious to casual observation. Calendered or clay coated papers on the other hand have a surface index of reflection which so differs from the coating that the coated areas can be seen.

Although this invention has been described with specific reference to its preferred embodiments, it is contemplated that modifications will occur to those skilled in the art and familiar with the principles herein set forth, and that such may be made without departing from the scope of this invention.

Having thus disclosed my invention and described in detail a preferred embodiment thereof, I claim and desire to secure by Letters Patent:

A self correcting testing device designed to receive marks from a pencil in selected areas corresponding to 10 a predetermined test pattern comprising a score sheet 20 having visible marks defining areas including said selected areas and also other areas outside of said test pattern, the surface of said selected areas of said sheet being of sufficient roughness and high frictional coefficient to receive a mark from a given pencil, and the surfaces of 25 said other areas being coated with a substance of sufficient smoothness and low frictional coefficient to resist marking from said pencil.

30 References Cited by the Examiner

UNITED STATES PATENTS

|           |         |                       |         |
|-----------|---------|-----------------------|---------|
| 1,849,708 | 3/1932  | Colbert et al. -----  | 35—66   |
| 1,883,775 | 10/1932 | Finkenbinder -----    | 35—48.1 |
| 1,884,197 | 10/1932 | Peterson et al. ----- | 35—26   |
| 2,210,879 | 8/1940  | Cahoon et al. -----   | 35—26   |
| 2,618,866 | 11/1952 | Adams -----           | 35—48.1 |

40 EUGENE R. CAPOZIO, Primary Examiner.

S. M. BENDER, R. W. WEIG, Assistant Examiners.